

2,734,862

## SYNTHETIC CASEIN FIBER ELASTIC GREASE

Arnold J. Morway, Rahway, N. J., and Robert P. Spray, Pittsburgh, Pa., assignors to Esso Research and Engineering Company, a corporation of Delaware

No Drawing. Application December 3, 1952,  
Serial No. 323,928

5 Claims. (Cl. 252—14)

The present invention relates to improvements in elastic fiber greases and particularly to improvements in the elasticity of the fibrous component thereof.

Fiber greases are widely used for packing certain types of journal bearings, for example, in railroad rolling stock. A relatively large quantity of such greases is consumed by industry. Such greases usually consist primarily of fibrous material such as wool fiber or yarn impregnated or saturated with an oil or grease composition. This lubricant is packed in a housing in such a way that it presses against the journal as it revolves and keeps it coated with a film of lubricant. The fiber or yarn acts as a reservoir for the oil or grease and prevents rapid consumption of the lubricant while assuring continuous lubrication.

In the prior art when the fibrous material, usually a reclaimed wool or yarn, has been used alone in combination with the lubricant it has tended to become matted and soggy and eventually to pull away from the bearing. This is particularly true when the bearings become heated up to temperatures of the order of 200° F. The oil rapidly evaporates and the fibers lose their resistance even if they are not actually charred. Upon failure of contact of the packing with the bearing there is a failure of lubrication with resulting damage to the bearing.

It has been proposed previously to maintain higher elasticity at ordinary temperatures in the conventional reclaimed wool fiber lubricant packing by inserting a coarser fiber such as horse hair, goat hair or other animal hair. The coarser and stiffer hair and the finer wool fibers are stranded and interspersed with each other and the entire fibrous mass is thereafter saturated with the oil or grease. While horse hair, in particular, has some utility in this connection at ordinary temperatures it is not particularly satisfactory as temperatures go above 150° F. or so and it is not always available. Horse hair and other animal hair fibers are also susceptible to actual damage at elevated temperatures and start to decompose and become brittle at temperatures as low as 150° to 180° F. They are therefore quite unsuitable at the moderately high journal and bearing temperatures frequently encountered in service, e. g., up to about 200° F. or sometimes a little higher.

According to the present invention it has been discovered that a relatively new type of synthetic fiber consisting of an extruded casein monofilament is a particularly suitable material for incorporation in elastic fiber greases which have a tendency to mat and lose contact with the bearing. This new synthetic fiber of coarse type has considerably greater elasticity than horse hair or the other coarse animal hairs and in particular it retains its elasticity much longer at moderately elevated temperatures. It is also more economical than horse hair, and related materials, and is readily available in increasing quantities. Furthermore, this material can be produced in any diameter and length desired and may readily be made either straight or curled.

For purposes of the present invention the curled extruded casein fiber of monofilament type is particularly suitable. Filaments which have been tested for purposes of the present invention have the following characteristics:

|                                      |                                |
|--------------------------------------|--------------------------------|
| Tenacity                             | 0.5—1.0 g./denier.             |
| Tensile strength                     | 8,500—16,000 p. s. i.          |
| Impact strength                      | 50—100 ft. lbs./sq. in.        |
| Knot strength                        | 5,000—7,500/sq. in.            |
| Diameter range                       | 0.005—0.016", 145—1330 denier. |
| Elongation at break                  | 20—25%.                        |
| Specific gravity                     | 1.29.                          |
| Moisture Regain:                     |                                |
| 65% RH 70° F                         | 10—15%.                        |
| 20% RH 70° F                         | 6.5%.                          |
| Burning rate                         | Very slow.                     |
| Resistance to heat                   | Some damage starts at 210° F.  |
| Resistance to abrasion               | Good.                          |
| Elastic recovery                     | Excellent.                     |
| Solubility in organic solvents       | Insoluble.                     |
| Color range                          | Unlimited (nat. color white).  |
| Resistance to mold, mildew and moths | Resistant.                     |

It will be seen from the foregoing that the curled casein monofilament of the type described above is particularly suitable for use in typical journal bearings where there is frequently some temperature elevation. A particular filament which is quite satisfactory is one which is sold under the trade name "Caslan." This "Caslan" fiber is becoming increasingly available and can readily be stranded with reclaimed wool, wool yarn or other available types of fiber.

It is preferred to combine the wool fiber and the casein fiber in proportions of about 75% wool (such as shredded carpet waste, for example) with about 25% by weight of the monofilament fiber. Proportions may be varied, however, from as little as 10% of the monofilament fiber to as much as 40%. It is always desirable to have a substantial portion of the finer wool fiber present for better wicking or capillary feed of the lubricant.

The lubricating ingredient itself is preferably a lubricating grease of soft consistency although an oil without a special thickener can be used in many applications. The composition presently preferred includes 75 to 95% by weight of calcium soap-mineral oil lubricating grease. Such a grease may contain from 3 to 20% of calcium soap of higher fatty acids such as the C<sub>12</sub> to C<sub>22</sub> saturated and unsaturated fatty acids. The soap may be prepared, of course, from substituted acids such as keto and hydroxy acids, for example, 4-keto-stearic acid or 12-hydroxy stearic acid, instead of fatty acids or in admixture therewith, if desired. Mixtures of soaps may be used and the soaps of other metals such as sodium, potassium, lithium, or aluminum may be employed. The calcium soap greases are usually less expensive and have a desirable consistency at usual journal bearing temperatures and they are normally preferred. Complex soaps of the soap-salt type may be used when high temperature grease stability is important.

Several examples were prepared in order to test out the invention. The first consisted of 85% by weight of a standard lime soap grease having a soap content of about 10 to 12% by weight. This is a soft, smooth, non-fibrous grease composition. To this was added 15% by weight, based on the total composition, of a mixture of wool waste obtained from shredded carpet and ordinary horse hair, the mixture containing about 25% horse hair and 75% wool.

A second sample was prepared exactly as in the first except that a monofilament casein fiber (curled "Caslan") was employed in lieu of the horse hair.

A third sample was prepared as in the case of Sample 2 except that the "Caslan" fiber was reduced to 10%, 90% of the fiber being wool waste.

A fourth sample consisted of 85% of the same lime soap grease as in Sample 1 with 15% of a blended fiber which contained 75% of long strand wool yarn and 25% "Caslan" fiber.

A fifth sample was the same as the fourth except that the "Caslan" fiber content was reduced to 10% of the total fibrous material.

It was observed in tests in journal bearings that 10% by weight of the "Caslan" was fully equivalent to 25% horse hair in imparting a good degree of elasticity to the fibrous material. All of the products described above were free from packing tendency but there was a greater degree of elasticity in the "Caslan" blended compositions than in others after holding them in an oven for 300 hours at 125 to 150° F.

In one test "Caslan" fiber was soaked in a mineral lubricating oil of relatively light viscosity (about 40 S. S. U. at 210° F.) for 3 months at a temperature which ranged between 150 and 250° F. There was no apparent deterioration of the "Caslan" fiber at the end of the test period. Also there did not appear to be any loss in elasticity over this extended period at the relatively high temperature range of 150 to 250° F. It will be appreciated that any fiber which tends to break down or become brittle at an operating temperature is quite unsatisfactory for industrial purposes. Even while being lubricated the journal bearings of railroad cars, for example, frequently become quite hot (200° F. or so) due to the heavy application of brakes to the wheels on long grades. The fibrous lubricating compositions of the present invention are substantially less susceptible to elastic deterioration at elevated temperatures than those of the prior art. They can be more closely controlled to obtain a desired degree of elasticity which may be maintained over a relatively long period of time. At the same time they are substantially less expensive than prior art compositions including horse hair. They are much more satisfactory in their resistance to packing or matting than standard fibrous lubricants which do not contain an elastic fiber.

It will be obvious that various types of oil, synthetic as well as mineral, may be used and that various thickeners may be used such as are used in the production of

lubricating greases and industrial oils. Furthermore, conventional anti-oxidants, extreme pressure additives, and the like may be incorporated as will be readily apparent to those skilled in the art.

What is claimed is:

1. An elastic fiber lubricant composition comprising a major proportion by weight of a lubricating grease and a minor proportion by weight of a fibrous mass comprising a major proportion of a mildly elastic wool fiber and about 10 to 40% by weight of a highly elastic extruded monofilament curled casein fiber, which has strong resistance against matting at temperatures up to at least 200° F.

15 2. An elastic fiber lubricant composition comprising 75 to 95% by weight of calcium soap-mineral oil lubricating grease and a fibrous mass comprising a major proportion of a relatively fine fiber wool waste, which has a tendency to become matted, and a minor proportion of a relatively coarse highly resilient extruded monofilament curled casein fiber sufficient to overcome said matting tendency.

25 3. Composition according to claim 2 wherein the casein fiber comprises 10 to 25% of the fibrous mass and is substantially unaffected by heat up to a temperature of about 210° F.

30 4. An elastic fiber lubricant composition consisting essentially of a fibrous mass impregnated with an oily lubricant, said mass comprising a major proportion of a wool fiber, which has a tendency to become matted, and a minor proportion of a curled, relatively coarse elastic extruded monofilament casein fiber interspersed through said mass to overcome said matting tendency.

35 5. Composition according to claim 4 wherein the oily lubricant is a calcium soap thickened mineral base lubricating oil.

#### References Cited in the file of this patent

##### UNITED STATES PATENTS

|            |         |               |
|------------|---------|---------------|
| 40 915,804 | Stearns | Mar. 23, 1909 |
| 1,001,371  | Drury   | Aug. 22, 1911 |
| 1,564,306  | Fantz   | Dec. 8, 1925  |
| 2,342,994  | Atwood  | Feb. 29, 1944 |

##### OTHER REFERENCES

45 Klemgard: "Lubricating Greases," Published 1937 by Reinhold Publishing Corp., 330 W. 42nd St., New York, N. Y., USA. Page 324.

50 Ser. No. 96,470, Ferretti (A. P. C.), published April 27, 1943.